

M. M. IRVINE,  
ELECTRODE AS USED FOR WELDING PURPOSES,  
APPLICATION FILED SEPT. 17, 1917.

1,261,395.

Patented Apr. 2, 1918.

*Fig. 1.*



*Fig. 2.*



Witnesses.

Geo. Marshall MacEachern.

Mary A. Lindsay.

INVENTOR.

Malcolm M. Irvine.

• F. J. Schubert  
ATTORNEY.

# UNITED STATES PATENT OFFICE.

MALCOLM M. IRVINE, OF GLASGOW, SCOTLAND.

## ELECTRODE AS USED FOR WELDING PURPOSES.

1,261,395.

Specification of Letters Patent.

Patented Apr. 2, 1918.

Application filed September 17, 1917. Serial No. 191,813.

To all whom it may concern:

Be it known that I, MALCOLM MILLER IRVINE, a subject of the King of Great Britain, residing at Glasgow, Scotland, have 5 invented certain new and useful Improvements Relating to Electrodes as Used for Welding Purposes, of which the following is a specification.

The object of the present invention is to 10 provide a tube of asbestos paper or pulp which is treated with iron, preferably in the form of an oxid and saturated with sodium carbonate and sodium silicate so as to give it distinctive properties when applied to a 15 metal rod or electrode as used in electric welding. The tubes may be made up separately and fitted on or to the rods when required or they may be formed or molded directly upon the rods used in welding.

20 The tubes are, preferably, made as follows, namely:—A layer or strip of asbestos paper sufficient to cover the required electrode is treated with appropriate quantities of iron oxid, sodium carbonate, and sodium silicate, and wound concentrically or spirally upon a metal rod or wire of standard gage or upon the actual welding wire.

25 In the treatment of the paper I, preferably, use the ingredients in or about the following proportions by weight, namely:—To every 100 parts of asbestos I add

|                  |           |
|------------------|-----------|
| Iron oxid        | 5 parts   |
| Sodium carbonate | 5 parts   |
| Sodium silicate  | 90 parts  |
| <hr/>            |           |
|                  | 100 parts |

35

In some cases in lieu of iron oxid, reduced iron in the form of a powder may be used.

40 It is to be understood the above proportions are merely given by way of example and they may, of course, be varied more or less as desired.

45 In some cases I may use asbestos pulp treated with the same ingredients as the paper after molding it into the form of a tube.

50 In order that the invention may be properly understood I have hereunto appended an explanatory drawing whereon I have, by way of example, shown an electrode provided with one of my flux tubes,

Figure 1 is a side elevation of the electrode, and

Fig. 2 a cross section thereof.

The electrode shown on the drawing consists of a welding wire *a* upon which is concentrically wound a piece of the treated asbestos paper *b* of suitable width and length.

Of course, instead of winding the paper concentrically into cylindrical form, as shown, it might be wound spirally. In this case I would use a long narrow strip of the treated asbestos paper and wind it spirally 65 around about the wire.

The method of treating the asbestos paper is preferably as follows:—The asbestos paper is cut of such a width as to give, when rolled on the molding wire, a thickness of 70 from 1 to 2 mm. The sodium carbonate and sodium silicate are dissolved in half their weight of hot water and mixed with the iron oxid. This mixture is then painted with a brush on to the asbestos. The liquid is absorbed while the iron oxid remains on the surface. The reverse side is then pasted or gummed so that the strip will adhere when applied to the wire. Alternatively the strip may be gummed to the wire and afterward dipped in the hot solution containing the sodium carbonate, sodium silicate and iron oxid. The coated wire is then heated 75 strongly to expel the water and destroy the paste. If the tube only is required it is removed by gripping it firmly in a suitable clamp and withdrawing the mandrel. In the case of an electrode the coating is dried 80 *in situ*.

The electrode provided with the flux tube 90 or coated in the manner before described produces the following changes during the process of welding. The primary arc is formed by the electrode itself and, at the high temperature, the external layer of oxid 95 is reduced to the metallic condition. A conducting ring of metal is thereby formed around the crater of the arc and, on the interruption of the primary arc by the dropping of the metal, continuity of arc is maintained by the external ring of metal. In this way a steady arc is insured so that a maximum welding speed may be attained 100 while the light emitted from the arc is yet

low and almost monochromatic and is, therefore, easily absorbed by the customary screens thus preventing the risk of eye troubles due to ultra violet light.

5. The electrode itself may be constituted by any special wire suited to the nature of the work.

The double arc makes it possible to obtain good welding results with alternating current and allows of greater latitude in the amount of current used so that the heat put into the work is more easily regulated.

Having now fully described my invention what I claim and desire to secure by Letters

15 Patent is:—

1. A tube, for use in electric welding, composed of asbestos paper or pulp treated with

iron (preferably in the form of an oxid) and saturated with sodium carbonate and sodium silicate, substantially as described. 20

2. A tube, such as claimed in claim 1, having the iron as an external coating.

3. An electrode for use in electric welding consisting of a metallic rod having thereon a flux tube composed of asbestos paper or 25 pulp treated with iron (preferably in the form of an oxid,) sodium carbonate and sodium silicate, substantially as described.

In testimony whereof I affix my signature in presence of two witnesses.

MALCOLM M. IRVINE.

Witnesses:

HUGH D. FITZPATRICK,

WILLIAM GALL.